

Jan. 2, 1951

J. W. OLSON

2,536,885

## METHOD OF MAKING MULTICONDUCTOR CABLES

Filed April 21, 1948



INVENTOR

BY  
Premier Edmund Winter & Barnes  
ATTORNEYS

## UNITED STATES PATENT OFFICE

2,536,885

## METHOD OF MAKING MULTICONDUCTOR CABLES

John W. Olson, Ardsley on Hudson, N. Y., assignor to Anaconda Wire and Cable Company, a corporation of Delaware

Application April 21, 1948, Serial No. 22,269

7 Claims. (Cl. 154—2.28)

1

This invention relates to insulated electrical cables, and is particularly concerned with the provision of an improved method of making multiconductor cables of the type known as "non-metallic sheathed cables" commonly used for building wiring. In accordance with the invention, the conductors are enclosed in a sheath made up of (1) a wrapping of fibrous material (preferably paper) which is precoated (but only on the side facing away from the conductors) with a thermoplastic composition, and (2) an overlying fibrous jacket impregnated with a thermoplastic composition under conditions that substantially prevent penetration of the thermoplastic material through the wrapping. The method of the invention leads to the production of a multiconductor cable of improved character, and such improved cables also come within the scope of this invention. This application is a continuation-in-part of my prior application Serial No. 542,720, filed June 29, 1944, entitled "Insulated Electrical Conductor", now abandoned.

Non-metallic sheathed cable usually comprises two or more wires each insulated with rubber and a bitumen-impregnated fibrous braid, and each wrapped with a folded-paper tape. The wires are enclosed in a sheath of fibrous material, generally in the form of a braided cotton jacket, with or without an underlying wrapping of paper. This sheath is impregnated with a bituminous saturant by immersing the sheathed cable in a heated molten bath of the saturant for a long enough period of time to saturate the jacket. The length of time required for saturation of the jacket, however, is necessarily also long enough for a substantial amount of the saturant to penetrate completely through the sheath (even when it includes a layer of paper immediately surrounding the insulated conductors), and cause the sheath to stick to the individual wires. This is a source of considerable annoyance and trouble to electricians who install the cable because it makes it difficult to separate and bare the conductors, without injuring the cable, for the purpose of making electrical connections. It also sometimes results in injury by overheating to wax finishers with which the paper tape wrappings about the individual conductors sometimes are impregnated, and even to the rubber insulation of the individual wires.

The improved method of the invention for manufacturing non-metallic sheathed cable and like multiconductor cables overcomes the foregoing disadvantages of the method heretofore

2

used, and leads to the production of an improved cable. In accordance with the invention, the individually insulated conductors are assembled together and a sheet of fibrous material such as paper, that has been precoated on one side only with a thermoplastic material, is wrapped about them. The wrapping is applied with its precoated side facing away from the conductors. A jacket of fibrous material, such as a cotton braid, is next applied over the wrapped assembly. Then the jacket is impregnated by immersing it in a thermoplastic material heated to a high enough temperature to be fluid. The duration of the impregnating operation is made long enough to effect saturation of the jacket, but is too short for any substantial amount of the thermoplastic material to penetrate through the wrapping. The precoating of the wrapping enables this control over the duration of the impregnating operation to be quite readily effected: the fibrous jacket in effect receives thermoplastic saturant from both sides, so that it becomes thoroughly saturated much more rapidly than by the method heretofore employed. The completed cable is characterized by having a well-impregnated jacket, but with the precoated wrapping free of any thermoplastic material on the side toward the conductors, so that the sheath is not stuck to the individual wires or to the paper tapes with which they are wrapped.

The thermoplastic material used in making multiconductor cables in accordance with the invention is preferably a bituminous composition having an A. S. T. M. ring and ball softening point above 125° F. and which is non-flowing at room temperature. The same composition may be used both for precoating the paper wrapping and for saturating the fibrous jacket, but better results can be obtained if the composition used for impregnating the jacket has a higher (by 50° F. or so) softening point than the material with which the wrapping is precoated. The actual duration of the impregnating operation is very short—not more than about five seconds and sometimes as short as one second or so when a bitumen having a softening point above 175° F. and heated to above 300° F. in the saturating bath is used for saturating the jacket.

The invention is described in greater detail below with reference to the accompanying drawing, the single figure of which shows a non-metallic sheathed cable made in accordance with the invention.

The cable shown in the drawing comprises a pair of metallic conductors 1 and 2, each having

an insulation made up of a layer of vulcanized rubber 3 and a covering of cotton braid 4 which is saturated with a thermoplastic material such as an asphaltic bitumen 5. The exterior of the insulation about one or both wires may be painted for purposes of circuit identification. Each of the insulated wires is provided with a spiral wrapping 7 of folded paper which serves to keep the wires out of contact with each other, and which makes the wires more readily accessible to electricians when the cable is installed. The individual wires are assembled side by side, and a filler of jute cord is laid in the valley spaces between them. The wires themselves and their assembly as thus-far described is conventional and does not by itself form any part of the present invention.

The assembly of individual wires and fillers is enclosed in a wrapping of fibrous sheet material 10 which has been precoated on one side only with a thermoplastic composition 11 such as an asphaltic bituminous composition. The wrapping 10 preferably is of crepe paper. It may be applied either as a spirally wound wrapping, or it may be in the form of a strip wrapped lengthwise around the assembled wires. In either case it is best applied with edges overlapping somewhat. The side of the wrapping to which the coating of bituminous material has first been applied faces away from the wires, and care should be taken to avoid crumpling the wrapping or otherwise deforming it in any manner that will bring its coated side into contact with the wires.

The precoating of bitumen or other thermoplastic material may be applied in any desired manner, using conventional paper-coating apparatus. An asphaltic bituminous coating may be applied either while heated to a thinly fluid condition, or in the form of a fluid emulsion. The coating should be dry and reasonably hard before the wrapping is applied about the assembled wires, in order to facilitate wrapping it in place.

An outer fibrous jacket 12 is applied over the wrapping 10. A cotton braid forms a particularly satisfactory outer jacket, but other fibrous materials such as spun glass, asbestos, or mixtures of these materials with each other or with cotton, may also be used.

After the outer jacket 12 has been applied, it is impregnated with an asphaltic bituminous composition or other thermoplastic material. Impregnation is accomplished most advantageously by immersing the jacketed assembly in a bath of the composition heated to a high enough temperature to be quite thinly fluid. It is characteristic of the method of the invention that the duration of the operation is very short—ordinarily not over about five seconds (in contrast to the time of five minutes or so required for complete saturation by methods heretofore employed). Five seconds or less has been found to be sufficient time to effect saturation of the jacket when the underlying paper wrapping has been precoated with an asphaltic bitumen, because the jacket in effect becomes impregnated from both sides at the same time. The jacket is not so thick but that the bituminous precoating on the wrapping 10 becomes softened enough to penetrate between the fibers of the jacket when the cable is immersed in a hot jacket saturant even for the short period of time the invention contemplates. As a result of the extremely short impregnation period, there is substantially no penetration of the bituminous composition through the paper wrapping and into contact with the

individual wires enclosed thereby. Hence these wires do not become stuck to the jacket, and the jacket is very readily removed wherever necessary for making electrical connections when the cable is installed. Furthermore, the very short impregnation period insures against any damage to the rubber and other materials forming parts of the insulation about the individual conductors 1 and 2—they do not become heated to any deleterious extent in so short a period of time. If, as is sometimes the practice, a coating of paraffin wax is applied to the insulated wires or to the folded-paper wrappings 7 thereabout, it comes through the impregnation step completely undamaged either in consequence of being overheated or by being fluxed with the bituminous material.

I prefer to employ a flame-resistant bituminous composition of the character described in the applications of John W. Olson and Charles W. Bechle Serial Nos. 415,144 (now U. S. Patent No. 2,442,706) and 415,145, (now U. S. Patent No. 2,442,707) filed October 15, 1941, both as the material with which the paper wrapping 10 is precoated and as the material with which the jacket 12 is saturated. Any bitumen used, however, should have a softening point above 125° F. Best results are secured when the bituminous material with which the jacket 12 is saturated has a higher softening point (preferably above 175° F.) than the coating 11 on the wrapping 10. As a specific example, very good results are obtained when using a flame-resistant asphaltic composition having a softening point of about 175° F. for precoating the wrapping 10, and a flame-resistant asphaltic composition having a softening point of about 225° F. for impregnating the jacket. The latter composition is heated to about 325° F. to render it adequately fluid for impregnation of the jacket, and the actual time of immersion of the jacketed cable in this hot saturating composition is only about a second or so.

Multiconductor cables having sheaths made in accordance with the invention are substantially as resistant to moisture absorption as similar cables made by the methods heretofore employed. They are superior to cables made by heretofore known methods in that the short period of immersion in the jacket-saturating bitumen insures against any damage to the vulcanized rubber or other components of the insulation about the individual wires, and in that the sheath is readily separated from the wires, without damage to the cable structure, wherever electrical connections must be made.

I claim:

1. In the manufacture of a multiconductor cable, involving assembling two or more wires within a common sheath, the improvement which comprises coating one side only of a sheet of fibrous material with a thermoplastic material, applying said coated sheet as a wrapping about an assembly of individually insulated wires with the coated surface of the sheet facing away from the wires, enclosing the thus-wrapped assembly in a fibrous jacket, and impregnating the jacket with a thermoplastic material heated to a high enough temperature to be fluid, the duration of the impregnating operation being long enough to effect saturation of the said jacket with the thermoplastic material but too short for any substantial amount of thermoplastic material to penetrate through said wrapping.

2. In the manufacture of a multiconductor cable, involving assembling two or more wires

within a common sheath, the improvement which comprises coating one side only of a sheet of fibrous material with a thermoplastic bituminous material that is non-flowing at room temperature, applying said coated sheet as a wrapping about an assembly of individually insulated wires with the coated surface of the sheet facing away from the wires, enclosing the thus-wrapped assembly in a fibrous jacket, and impregnating the jacket with a thermoplastic bituminous material heated to a high enough temperature to be fluid, the duration of said impregnating operation being long enough to soften the bituminous coating on the wrapping and effect saturation of the jacket with the bituminous material but too short for any substantial amount of the bituminous coating on the wrapping to penetrate therethrough.

3. In the manufacture of a multiconductor cable, involving assembling two or more wires within a common sheath, the improvement which comprises forming said sheath by applying about an assembly of individually insulated wires a wrapping of fibrous sheet material that has been precoated on one side only with a bituminous material having a softening point above 125° F., said wrapping being applied with its coated side facing away from the wires, applying a jacket of fibrous material about the thus-wrapped assembly, and impregnating the jacket with a bituminous material having a softening point above 125° F. and heated to above said softening point, the duration of the impregnating operation being long enough to soften the bituminous coating on the wrapping and effect saturation of the jacket with the bituminous material but too short for any substantial amount of the bituminous material to penetrate through the wrapping.

4. In the manufacture of a multiconductor cable, involving assembling two or more wires within a common sheath, the improvement which comprises forming said sheath by applying about an assembly of individually insulated wires a wrapping of paper that has been precoated on one side only with a bituminous material having a softening point above 125° F., said paper being applied with its coated side facing away from the wires, applying a jacket of fibrous material about the thus-wrapped assembly, and immersing the jacketed assembly in a bituminous material having a softening point above 125° F. and heated to above said softening point for a period of time long enough to soften the bituminous coating on the paper wrapping and effect saturation of the fibrous jacket with the bituminous material but too short for any substantial amount of the bituminous material to penetrate through the paper wrapping.

5. In the manufacture of a multiconductor cable, involving assembling two or more wires within a common sheath, the improvement which comprises forming said sheath by applying about an assembly of individually insulated wires a wrapping of paper that has been precoated on one side only with a bituminous material having a softening point above 125° F., said paper being applied with its coated side facing away from the wires, applying a jacket of fibrous material about the thus-wrapped assembly, and immersing the jacketed assembly in a bituminous material hav-

ing a softening point above 125° F. and heated to above 300° F. for a period of time not longer than about five seconds, whereby the coating on the paper is softened and the fibrous jacket is impregnated with the bituminous material but no substantial amount of the bituminous material penetrates through the paper.

6. In the manufacture of a multiconductor cable, involving assembling two or more wires within a common sheath, the improvement which comprises forming said sheath by applying about an assembly of individually insulated wires a wrapping of fibrous material that has been precoated on one side only with a first thermoplastic material, said wrapping being applied with its coated side facing away from the wires, applying a jacket of fibrous material about the thus-wrapped assembly, and impregnating the jacket with a second thermoplastic material having a softening point higher than that of said first thermoplastic material and heated to a temperature above its softening point, the duration of the impregnating operation being long enough to soften the first thermoplastic material coating the wrapping and effect saturation of the jacket with the thermoplastic materials but too short for any substantial amount of bituminous material to penetrate through the fibrous wrapping.

7. In the manufacture of a multiconductor cable involving assembling two or more wires within a common sheath, the improvement which comprises forming said sheath by applying about an assembly of individually insulated wires a wrapping of paper that has been precoated on one side only with a first bituminous material having a softening point above 125° F., said wrapping being applied with its coated side facing away from the wires, applying a jacket of fibrous material about the thus-wrapped assembly, and impregnating the jacket with a second bituminous material having a softening point higher than said first bituminous material and above 175° F. by immersing the jacketed assembly for a period not longer than about five seconds in a bath of said second bituminous material that is heated to a temperature above 300° F., whereby the coating on the paper wrapping is softened and the jacket is thoroughly saturated with bituminous material but no substantial amount of the bituminous material penetrates through the paper wrapping into contact with the individual insulated wires.

JOHN W. OLSON.

#### REFERENCES CITED

The following references are of record in the file of this patent:

#### UNITED STATES PATENTS

| 60 | Number    | Name            | Date           |
|----|-----------|-----------------|----------------|
|    | 809,312   | Lougee          | Jan. 9, 1906   |
|    | 1,890,253 | Frederickson    | Dec. 6, 1932   |
|    | 1,905,789 | Benner et al.   | Apr. 25, 1933  |
|    | 2,090,510 | Bower           | Aug. 17, 1937  |
| 65 | 2,093,411 | Bowden et al.   | Sept. 21, 1937 |
|    | 2,222,638 | Szilard         | Nov. 26, 1940  |
|    | 2,281,111 | Robinson et al. | Apr. 28, 1942  |
|    | 2,426,413 | Pollett         | Aug. 26, 1947  |